

1,261,366.

E. DANNER.  
METHOD OF FORMING SHEET GLASS.  
APPLICATION FILED MAY 3, 1916.

Patented Apr. 2, 1918.

6 SHEETS—SHEET 1.

Fig. 1.



INVENTOR  
Edward Danner,  
By C. Wm. Owen & Crampton,  
His Atty.

1,261,366.

E. DANNER,  
METHOD OF FORMING SHEET GLASS.  
APPLICATION FILED MAY 3, 1916.

Patented Apr. 2, 1918.  
6 SHEETS—SHEET 2.

Fig. 2.



3 23 INVENTOR

Edward Danner,  
By C. W. Crampton,  
His attys.

E. DANNER.  
METHOD OF FORMING SHEET GLASS.  
APPLICATION FILED MAY 3, 1916.

1,261,366.

Patented Apr. 2, 1918.  
6 SHEETS—SHEET 3.

FIG. 3.



1,261.366.

E. DANNER.  
METHOD OF FORMING SHEET GLASS.  
APPLICATION FILED MAY 3, 1916.

Patented Apr. 2, 1918.  
6 SHEETS—SHEET 4.

Fig. 4.



Fig. 6.

Fig. 5.



INVENTOR  
Edward Danner,  
By Burn, Burn & Crampstone.

E. DANNER.

METHOD OF FORMING SHEET GLASS.

APPLICATION FILED MAY 3, 1916.

1,261,366.

Patented Apr. 2, 1918.

6 SHEETS—SHEET 5.



FIG. 8

INVENTOR

Edward Danner,

By Own. Own & Crampton,  
His atty.

E. DANNER.

METHOD OF FORMING SHEET GLASS.

APPLICATION FILED MAY 3, 1916.

1,261,366.

Patented Apr. 2, 1918.

6 SHEETS—SHEET 6.

FIG. 9.  
FIG. 10.



INVENTOR

Edward Danner,

By Burn, Burn & Crampton,  
his atty.

# UNITED STATES PATENT OFFICE.

EDWARD DANNER, OF TOLEDO, OHIO.

## METHOD OF FORMING SHEET-GLASS.

1,261,366.

Specification of Letters Patent.

Patented Apr. 2, 1918.

Application filed May 3, 1916. Serial No. 95,070.

To all whom it may concern:

Be it known that I, EDWARD DANNER, a citizen of the United States, and a resident of Toledo, in the county of Lucas and State of Ohio, have invented a certain new and useful Method of Forming Sheet-Glass; and I do hereby declare the following to be a full, clear, and exact description of the invention, such as will enable others skilled in the art to which it appertains to make and use the same, reference being had to the accompanying drawings, and to the characters of reference marked thereon, which form a part of this specification.

15 This invention relates to the glass working art and particularly to the manufacture of sheet glass, and has for its object the provision of an improved method for continuously forming molten glass in sheet form 20 in a rapid, efficient and economical manner and without the use of pressing or sizing rolls.

25 The invention is fully described in the following specification, and while, in its broader aspect, it is capable of being practised by numerous apparatus, a few only of such apparatus are illustrated in the accompanying drawings, in which—

Figure 1 is a side elevation of one form of apparatus for practising my invention, with a part of the furnace broken away. Fig. 2 is a front end elevation thereof, with a part broken away. Fig. 3 is a section on the line 3—3 in Fig. 2, with glass being drawn in sheet form therefrom. Fig. 4 is a section on the line 4—4 in Fig. 3, with a part broken away. Fig. 5 is an enlarged side elevation of a portion of the apparatus illustrating the slab adjusting means. Fig. 6 is a section on the line 6—6 in Fig. 5. Fig. 7 is a sectional view of a portion of the apparatus illustrating a slightly modified form of the slab. Fig. 8 is a front end elevation of a different form of apparatus for practising the invention. Fig. 9 is a section thereof on the line 9—9 in Fig. 8. Fig. 10 is a section on the line 10—10 in Fig. 9, and Fig. 11 is a partial sectional view of the apparatus with a different form of drawing slab from that illustrated in Figs. 8 to 10 inclusive.

55 The practising of my invention in its broad aspect, contemplates distributing molten glass evenly on a slab which is disposed in a heated chamber, and drawing the glass in sheet form off the slab to stretch it to the desired thickness. For the practical

and satisfactory drawing of sheet glass by my process it is important to maintain the slab, on which the glass is first distributed and from which it is drawn in sheet form, 60 highly heated so that the molten glass in flowing down the same is not permitted to too quickly cool, and also to maintain the slab, or at least a greater portion thereof, in a high temperature so as to retard the 65 external cooling of the glass surface as it flows down and is drawn from the slab.

In the apparatus illustrated in Figs. 1 to 6, 1 designates a furnace containing molten glass 2, which flows from the furnace 70 over a trough 3 into a practically closed chamber 4, that is heated by flames from a plurality of burners 5, if gas is employed as a fuel, which burners are arranged in suitable positions within said chamber. The 75 trough 3 terminates within the chamber 4 and the flow of molten glass from its discharge end is regulated by a gate 6, which, for such purpose, is suitably mounted for vertical adjustment in the chamber 4 with 80 respect to the trough.

The molten glass is intended to flow in a comparatively thin broad stream from the outer end of the trough 3 down onto the upper surface of a slab 7, which is disposed in 85 subjacent relation to the discharge end of the trough and rearwardly inclined to permit the glass to flow down the same in sheet form. The glass as it flows down the slab 7 is partially cooled from the molten state 90 in which it flows from the trough 3 to give the glass sufficient consistency to enable it to be continuously drawn off in sheet form from the lower discharge end of the slab. Any suitable means not shown may be provided for imparting a continuous drawing 95 movement to the glass sheet A, the speed of drawing being regulated to suit the thickness of the glass sheet required and the free-ness with which the glass flows down and 100 from the outer end of the slab 7. It will be understood that the drawing of the glass from the slab causes the glass sheet to be stretched to the desired thickness instead of utilizing sizing rolls for such purpose, 105 as has heretofore been the practice. Side pieces 7<sup>a</sup> are mounted on the top of the slab 7 adjacent to its side edges and are adjustable to determine the width of the glass sheet, and to serve as a guide to prevent 110 the glass from spreading while flowing down the slab.

In order that the temperature within the portion of the chamber 4 in which the slab 7 is disposed may be regulated to suit the conditions of drawing, which conditions 5 vary for sheets of glass of different thickness, adjustable gates are provided above and below the discharge end portion of the slab 7 and may be adjusted inward and outward to vary the size of the opening through 10 which the slab 7 projects and also to expose a greater or less portion of the slab to the outside atmosphere or to a temperature less than that of the chamber 4. The upper gate is designated 8 and is hingedly connected, as at 9, to a vertically movable plate 10 forming a portion of the front of the chamber 4 and also has rack-bar-and-pinion connection 11 with a shaft 12 that is carried by the plate 10 through the medium of 20 bracket arms 13, thus adapting a turning of the shaft 12 to effect an inward or outward swinging of the gate 8 with respect to the slab 7. The lower gate 14 has rack-bar-and-pinion connection 15 with a shaft 25 16 mounted in the lower frame 17 of the apparatus, whereby a turning of said shaft will effect a substantially vertical or lengthwise movement of the gate 14. The upper end of the gate 14 has a link 18 projecting 30 from each end thereof within the chamber 4 below the slab 7 and a rack bar and pinion 19 (Fig. 6) connects each link to a shaft 20, whereby a turning of such shaft effects an inward and outward swinging movement of 35 the gate 14, as is apparent.

The slab 7 is hung at its rear end on the shaft 20 for adjusting movements about the same as an axis, and is adjustably supported at its forward end by a plurality of rods 21, 40 which are mounted on the outer side of the gate 14 and guided for vertical movements thereby. The lower end portions of these rods thread through respective nuts 22, fixed to the gate 14 and the several rods have 45 chain and sprocket connection 23 with each other, as best shown in Fig. 2. It is evident that a turning of the rods 21 will effect a vertical movement thereof and cause a raising or lowering of the outer or forward end 50 of the slab 7, and will increase or decrease the opening between the slab 7 and the gate 14, this tilting of the slab and regulation of opening being desirable to meet the conditions and temperature of the glass being 55 worked.

In Fig. 7 the slab on which the glass flows from the trough 3 is designated 24 and has the surface thereof over which the glass flows vertically disposed to permit the downward drawing of the glass sheet therefrom in a vertical plane. In this case the upper end portion of the surface of the slab on which the glass flows is rearwardly offset from the vertical portion of such surface 60 and stands in position for the molten glass 65

2, as it flows from the trough 3, to fall thereon, the glass then being distributed in sheet form over the surface of the slab and flowing downward therefrom. The glass sheet is drawn from the lower end of the slab 24, the speed of drawing being so regulated with respect to the speed of flow of the glass down the face of the slab 24 as to effect the desired sizing of the sheets. It is evident that with this form of slab the surrounding 70 temperature would need to be less than that required if the slab was inclined, as otherwise the glass would flow too freely down the vertical slab 24.

In the form of apparatus illustrated in 80 Figs. 8, 9 and 10 for practising the invention the slab is vertically disposed and the molten glass is caused to flow down the same in a regulated stream which entirely surrounds or encompasses the slab. In this apparatus the trough 3 in which the molten glass flows from the furnace 1 terminates at its outer end in a pot or tank 25, that is disposed within a heating chamber 26, which is heated, in the present instance, by flames 90 from a plurality of gas burners 27. The pot 25 is elongated transversely of the trough 3 to suit the width of the glass sheets to be drawn and is provided at its bottom with an elongated opening 28, which extends substantially the length of the pot 25. A slab 29 of corresponding shape in cross-section to the opening 28 projects down through the opening and into a heating chamber 30, which is formed immediately below the bottom of the pot 25 by a wall 31.

The slab 29 is carried by hollow stems or tubes 32, which project up through the pot and the top of the heating chamber 26, being provided above said top with sprocket-wheels 33, which are threaded on the stems and rest at the lower ends of their hubs on a cross-beam 34 at the top of the furnace. The sprocket wheels 33 are connected by a sprocket-chain 35, and one also has chain 110 and sprocket connection 36 with an adjusting shaft 37, whereby a turning of said shaft will effect a uniform turning of the sprocket wheels 33 and a vertical adjusting of the slab 29. The head portion 29a of 115 the slab 29 has its side walls outwardly and upwardly inclined whereby a raising or lowering of said head within the outlet opening 28 of the pot effects a variation in the size of such opening to regulate the flow of 120 molten glass from the pot.

The lower end of the chamber 30 is open to permit the flames from a burner 38 to pass upward therein from below the same and around the glass that is flowing down 125 the slab 29. The flames and gases within the chamber 30 find an exit from the upper end thereof through a plurality of openings 39 in its wall. It is thus evident that the flame from the burner 38, or the heat gen-

erated thereby, which rises around the glass as it flows downward from the pot 25 through the chamber 30, retards the cooling of the glass and permits it to be drawn 5 from the lower end of the slab 29 and sized as to thickness by the drawing action. If the lower end of the slab 29 is broad or terminates with the side terminal spaced, as shown, and air a little above atmospheric 10 pressure is supplied to the interior of the drawn glass through the slab 29, the glass will be drawn in transversely elongated hollow form, as shown at B, with the opposing side walls thereof parallel and connected by 15 short end portions. In such case the short curved end portions of the drawn glass are severed from the side walls in any suitable manner, which forms no part of the present invention and will therefore not be described, thus severing the drawn glass into 20 two separate sheets of uniform thickness and quality.

If the lower end of the slab 29 is made V-shape in cross-section, as shown at 29<sup>b</sup> 25 (Fig. 11), the glass which flows down the slab at the opposite sides thereof will merge at the lower end of the slab into a single sheet C, which is drawn to proper size after leaving the slab.

30 It is evident in the use of each of the apparatus shown and described that the molten glass is caused to flow in a molten state down a heated slab disposed in a heated chamber, the glass being distributed over 35 the slab and flowing down and from the same in sheet form, either single or multiple, the flowing of the glass from the slab being augmented by mechanical means which causes a stretching out and thinning or sizing 40 of the sheet after leaving the slab. It will be understood that the thickness of the drawn sheet is dependent not only on the speed of drawing of the sheet from the slab, but also on the quantity of flow of molten 45 glass from the trough 3 or pot 25, as the case may be, down the slab, and on the temperature maintained in the chamber within 50 which the slab is disposed, it being evident that the lower the temperature within the slab chamber the more quickly will the glass harden and set. As the glass sheet is drawn 55 from the slab and becomes hardened it is severed into sections by any suitable means, such severing means not being illustrated herein, as it forms no part of the present invention. Such severing, however, should take place at the outer side of the drawing means so that the drawn glass sheet will be 60 continuously maintained between the slab and the drawing means.

By the use of my process the use of the sizing rolls heretofore commonly employed is obviated, thereby preventing or overcoming the rough surfaces of glass sheets occasioned by the rolling process. A further

and very important feature of my process over those heretofore employed for making sheet glass is the increased speed with which the glass can be drawn and the uniformity in thickness of the product.

I wish it understood that the forms of apparatus herein described and shown for practising my invention are made merely for the purpose of illustration and not to restrict the scope of the invention as defined 70 in the claims, and that the process is not limited to use in connection with any particular apparatus.

Having thus described my invention, what I claim as new, and desire to secure by Letters Patent, is,—

1. The method of forming sheet glass, consisting in permitting molten glass to flow down a slab in the presence of heat, and drawing the glass from the slab.

2. The method of forming sheet glass, consisting in permitting molten glass to flow by gravity down a member disposed in a heated atmosphere and having a flat surface, and drawing the glass from the lower 90 end of said member.

3. The method of forming sheet glass, consisting in permitting molten glass to flow down a heated slab in the presence of heat, and continuously drawing the glass from 95 the lower end of the slab.

4. The method of forming sheet glass, consisting in permitting molten glass to flow down a slab in the presence of heat, and applying a continuous predetermined pull 100 on the glass after passing from the slab to size the same.

5. The method of forming sheet glass, consisting in permitting molten glass to flow by gravity down a heated slab in the presence of heat and augmenting the gravity movement of the glass by applying a continuous predetermined outward drawing pull thereto after leaving the slab, which pull stretches the glass to predetermined 110 thickness.

6. The method of forming sheet glass, consisting in flowing glass in a molten state down a heated slab and stretching it therefrom to predetermined thickness.

7. The method of forming sheet glass, consisting in flowing glass in a molten state down a heated slab and in a heated atmosphere to flatten and retard the cooling thereof, and applying a stretching pull to 120 the glass after leaving the slab to size it.

8. The method of forming sheet glass, consisting in permitting molten glass to flow in a regulated stream down a slab in the presence of heat, and drawing the glass from 125 the slab.

9. The method of forming sheet glass, consisting in permitting molten glass to flow by gravity in a regulated stream down a slab in the presence of heat, and drawing 130

the glass from the lower end of said slab to stretch it to predetermined thickness.

10. The method of forming sheet glass, consisting in permitting molten glass to flow in a regulated stream down a heated slab in the presence of heat, and continuously drawing the glass from the lower end of the slab to stretch it to predetermined thickness.

11. The method of forming sheet glass, 10 consisting in supplying glass in evenly distributed form to the surface of a slab at the rear of its discharge end and in the presence of heat, the glass flowing down the slab by gravity and being drawn from its discharge end to stretch the glass to predetermined size.

12. The method of forming sheet glass, 20 consisting in permitting molten glass to flow down a slab over the surface thereof toward its discharge end, and constantly drawing the glass therefrom at a predetermined speed to stretch it to the desired thickness, said stretching taking place from the time the glass leaves the slab until it is in a set condition.

13. The method of forming sheet glass, 30 consisting in permitting molten glass to continuously flow in a regulated stream down a heated slab in the presence of heat, and constantly drawing the glass from the discharge end of the slab at a predetermined speed to stretch it to the desired thickness, said stretching continuing from the time the glass leaves the slab until it is in a set condition.

14. The method of forming sheet glass, 40 consisting in causing molten glass to be continuously and evenly distributed over the surface of a slab above its discharge end, to flow down the same by gravity, and to be constantly drawn from the discharge end thereof at a predetermined speed to stretch it to the desired thickness, said stretching taking place from the time the glass leaves the slab until it is in a set condition, and before reaching the drawing means.

15. The method of forming sheet glass, 50 consisting in permitting molten glass to flow down a heat surrounded slab, and drawing the glass from the slab, the heat being less at the portion of the slab from which the glass is drawn than at the point of flow of the glass thereon.

16. The method of forming sheet glass, 55 consisting in providing a slab within a heated chamber and projecting the discharge end thereof into a temperature which is less than that of the chamber, and causing molten glass to flow onto the slab within the chamber and to be drawn from the discharged end thereof.

17. The method of forming sheet glass, 60 consisting in flowing glass in a molten state over an inclined heated slab and stretching it from the lower end thereof in sheet form

to predetermined thickness before the sheet reaches the stretching means.

18. The method of forming sheet glass, 70 consisting in permitting molten glass to flow down an inclined slab in the presence of a surrounding heat, and drawing the glass from the slab, the heat being less at the portion of the slab from which the glass is drawn than at the point of flow of the glass thereon.

19. The method of forming sheet glass, 75 consisting in providing an inclined slab within a heated chamber and projecting the outer end thereof into a temperature which is less than that of the chamber and causing molten glass to flow onto the slab within the chamber and to be drawn from the discharge end of the slab the drawing stress being applied to the sheet beyond the point of set.

20. The method of forming sheet glass, 80 consisting in permitting molten glass to flow in a regulated stream onto and down a heated slab in the presence of a surrounding heat and drawing the glass from the slab, 90 the heat diminishing from the portion of the slab on which the glass first flows to the portion thereof from which the glass is drawn, the drawing stress being applied beyond the point of set of the sheet.

21. The method of forming sheet glass, 95 consisting in permitting molten glass to flow down a heated slab in the presence of heat, drawing it therefrom to predetermined thickness and regulating the width 100 of flow of the glass down the slab.

22. The method of forming sheet glass, 105 consisting in permitting molten glass to flow by gravity from a trough down onto an inclined slab in a broad regulated stream, the glass then flowing down the slab and being drawn from its lower end at a predetermined speed to stretch it to the desired thickness, the width of the glass column as it flows down onto the slab being 110 substantially the same as the width of the sheet drawn from the slab, and the drawing stress being applied beyond the point of set of the sheet.

23. The method of forming sheet glass, 115 consisting in permitting molten glass to continuously flow in a regulated stream down onto a slab, the flow down the slab being by gravity, and drawing the glass from the slab at a speed which is greater 120 than the speed of flow of the glass onto the slab whereby the glass is stretched to predetermined thickness before reaching the drawing means.

24. The method of forming sheet glass, 125 consisting in causing molten glass to continuously flow onto, down and from a slab in sheet form and subjecting the sheet, as it flows from the slab, to a continuous uniform longitudinal stretching stress applied 130

thereto beyond the point where the glass becomes set.

25. The method of forming sheet glass, consisting in causing molten glass to continuously flow onto, down and from a slab in sheet form and in the presence of a surrounding heat and subjecting the sheet, as

it flows from the slab, to a continuous uniform longitudinal stretching stress applied thereto beyond the point where the glass becomes set.

In testimony whereof, I have hereunto signed my name to this specification.

EDWARD DANNER.